

May 1, 1923.

1,453,382

D. D'ALESSANDRO ET AL

METHOD OF MAKING TILES

Filed Nov. 3, 1922



Inventors  
Dominick DiAlessandro  
Raffaele Pace  
by David Rines  
Attorney

Patented May 1, 1923.

1,453,382

# UNITED STATES PATENT OFFICE.

DOMINICK D'ALESSANDRO AND RAFFAELE PACE, OF QUINCY, MASSACHUSETTS; SAID PACE ASSIGNOR TO SAID D'ALESSANDRO.

## METHOD OF MAKING TILES.

Original application filed March 1, 1921, Serial No. 448,900. Divided and this application filed November 3, 1922. Serial No. 598,720.

To all whom it may concern:

Be it known that we, DOMINICK D'ALESSANDRO and RAFFAELE PACE, respectively a citizen of the United States and a subject 5 of the King of Italy, and residents of Quincy, in the county of Norfolk and Commonwealth of Massachusetts, have invented a new and useful Improvement in Methods of Making Tiles, of which the following is a specification.

10 The present application is a division of application Serial No. 448,900, filed March 1, 1921.

This invention relates to methods of manufacturing cement or concrete articles, like 15 tiles, and it has for its object to improve upon present-day methods of the above-designated character, to the end that a superior article may be produced more economically and efficiently.

With this end in view, the invention consists of the improved method a preferred embodiment of which is hereinafter described, 20 illustrated in the accompanying drawings, and defined in the appended claims.

In the drawings, Fig. 1 is a vertical section, illustrating the present invention; Fig. 2 is a view illustrating the removal of a tile 25 from the mold; Fig. 3 is a plan view of the removable walls of a mold that may be used in carrying out the method of the present invention; Fig. 4 is a similar view of the bottom wall of the mold; Fig. 5 is a view of 30 a color pattern; and Fig. 6 is a section taken upon the line 6—6 of Fig. 5, looking in the direction of the arrows.

The illustrative mold comprises a plate 2, the upper face 4 of which constitutes the bottom wall of the mold, and two members 6 and 8, the inner faces 10 and 12 of which constitute the side walls of the mold. The member 6 is provided with extensions 14 and 16, and the member 8 with similar extensions 40 18 and 20 that respectively abut against the extensions 14 and 16 of the member 6. A bolt 22 loosely secures the extensions 14 and 18 together to permit a slight pivotal movement of the members 6 and 8 towards and 45 from each other. The extension 20 is perforated, and through the perforation 24 extends a lug 26 mounted upon the extension 16. The lug 26 is preferably a bolt, as shown. A cam lever 28 is pivoted to the

free end 30 of the lug 26 and is adapted to 55 engage the perforated extension 20 to force the members 6 and 8 towards each other and secure them firmly in such position.

The side edges 32 of the plate 2 are provided with lugs 34 upon which the members 60 6 and 8 are adapted to rest. As will be clear more particularly from Fig. 1, the lugs 34 are positioned below the bottom wall 4 of the mold, so that the side walls 10 and 12 may firmly and tightly engage the side edges 65 32 when the members 6 and 8 are forced towards each other by the cam lever 28. A pivotal movement of the cam lever 28 in the opposite direction will permit slight pivotal separation of the side walls 10 and 12, about 70 the bolt 22, away from the side edges 32, permitting the removal of the members 6 and 8 from the lugs 34. The members 6 and 8, and the side walls 10 and 12 of the mold formed thereon, are thus easily removable as a unit from the bottom wall of the mold, and are as readily returnable thereto.

The term "tile" will be employed throughout the specification and the claims 80 to designate tiles and similar cement articles, whether or not used as tiles. To manufacture tiles according to the method of the present invention, the side walls of the mold are first assembled, as above described, upon 85 the bottom wall. A very thin surface layer of liquid cement, indicated in the drawings by a heavy line 36, is then poured upon the bottom wall. This surface layer should not be too thin, because it would then wear very 90 rapidly away from the face of the completed tile; and it can not be too thick, else the different colored portions of this surface layer (if different colors are employed) would overrun into one another when the 95 pattern shown in Figs. 5 and 6 is removed, as described below. For lack of a better term, this thin surface layer 36 will herein-after be referred to in the specification and the claims as a "film-like" layer. Care 100 should be taken to spread this film-like, surface layer 36 uniformly on the bottom wall 4, as by oscillating the mold back and forth several times until the layer has spread evenly. This film-like layer is preferably 105 composed of suitable proportions of very fine sand and very fine cement with a plentiful proportion of water or other liquid added

thereto to render it very liquid. The term "cement" will, for brevity, be employed throughout the specification and the claims to denote cement or sand or any suitable mixture of them or their equivalents, and the term "liquid cement" will be similarly employed to denote the same with a liberal proportion of water or other liquid added thereto. This layer may be colored, if desired, by the addition of some suitable coloring material.

A thin layer of fine, very dry, granular cement, consisting, preferably, of a mixture of two parts fine cement and one part fine sand, is then introduced over the liquid cement. This layer is indicated in Fig. 1 by the numeral 38. The dry layer 38 absorbs the liquid of the liquid layer 36, but the ingredients thereof are so fine as not to protrude noticeably through the liquid layer to the surface. The surface of the completed tile would be marred by such protrusion if the layer 38 were composed of coarse materials, particularly if the surface layer 36 is colored.

A layer 40 of coarse, moist cement, constituted preferably of two parts coarse sand and one part coarse cement, is then introduced over the layer 38 of the fine dry cement. The layer 40 is thick, according to the dimensions of the desired tile. A cover plate 42, having an upper mold wall 44, is placed in position upon the coarse layer 40, and is driven home under great pressure.

The cam lever 28 is then manipulated to permit removal of the members 6 and 8, after which the cover plate 42 is removed by means of handles 54 that are integrally secured to the cover plate. The pressed tile, though well formed is still somewhat weak, so requires support during its removal from the bottom wall 4. This support is preferably obtained by placing over it a previously completed tile 56. A plate 58 is positioned along the edge of the tile, and grasped in one hand, as shown in Fig. 2, a handle 60 that is integral with one of the lugs 34 is grasped in the other, and a sidewise thrust in the direction of the arrow is exerted by the one hand towards the other hand to thrust the tile sidewise off the bottom wall 4 of the mold. The plate 2 may, if desired, be tilted at such time, as illustrated in Fig. 2. The tile is then allowed to rest for a period, preferably upon the tile 56, after which it is immersed in water and allowed to harden or set properly.

The use of the liquid, film-like, surface layer 36 is particularly desirable in the preparation of tiles having smooth or colored surfaces. The liquid layer, however, has a tendency to stick to the bottom wall 4 of the mold, causing breaking up of the surface of the tile when it is attempted to remove the tile from the mold. The bottom

wall 4 must, therefore, be suitably lubricated or oiled before the liquid layer is poured thereon. Lubricants, however, are liable to cause grease spots upon the surface of the tile, and they have a tendency to contract, causing the surface of the hardened tile to crack. According to the present invention, these difficulties are eliminated by the use of a lubricant containing a grease-absorbing element, such as turpentine or kerosene, and an element for preventing the formation of cracks in the surface of the completed tile, as olive oil.

In the manufacture of tiles the surfaces of which are variously colored, it is essential that the lines of separation between the colors be sharp and that the designs be properly centered. The design may, for example, be like that of the pattern shown in Fig. 5, or it may be very much simpler, as a single dividing line. The pattern is placed upon the bottom wall 4 and a film-like surface layer of differently colored liquid cements is poured upon the bottom wall between the walls of the pattern. The color between the walls 64 may, for example, be red; that between the walls 66 green; that along the sides, between and under the walls 68, white; and that along the corners, between the walls 70, of still another color. After the film-like surface layer has been uniformly spread over the bottom wall, as above described, the pattern is removed to permit the differently colored liquid cement to flow towards each other and form sharp, dividing lines of demarcation. The rest of the process is as above described.

It is essential that the pattern be removed before the fine layer 38 is applied, for if the latter is introduced while the pattern is still in position, the dry cement, after absorbing liquid from the film-like, liquid, surface layer, will stick to the walls of the pattern, so that upon removal of the pattern, the differently colored layers will flow into one another, forming a jagged line of demarcation.

To correctly center the design, the pattern is provided with exterior walls 72 of dimensions equal to the dimensions of the mold, so that the walls 72 may contact with the side walls 10 and 12 of the mold, maintaining the pattern properly positioned within the mold. Bars 74 rigidly connect the walls of the pattern to the exterior walls 72, but are spaced from the bottom wall 4, as will be clear from Fig. 6, so as not to interfere with the flow of the colored film-like layer under the bars 74.

It will be obvious to persons skilled in the art that the details of the invention may be varied from what is shown and described herein, and such variations are considered to be within the spirit and scope of the invention, as defined in the appended claims.

What is claimed as new is:

1. The method of making tiles that comprises successively positioning a pattern upon the bottom wall of a mold, pouring a film-like surface layer of differently colored liquid cements upon the bottom wall between the walls of the pattern, removing the pattern to permit the differently colored liquid cements to flow towards each other and form sharp dividing lines of demarcation, introducing a layer of granular cement over the liquid cement and subjecting the whole to pressure.
2. The method of making tiles in a mold having bottom and side walls that comprises successively positioning a pattern upon the bottom wall with a portion thereof in contact with a side wall to maintain the pattern properly positioned within the mold, pouring a film-like surface layer of differently colored liquid cements upon the bottom wall between the walls of the pattern, removing the pattern to permit the differently colored liquid cements to flow towards each other and form sharp dividing lines of demarcation, introducing a layer of fine, dry cement over the liquid cement to cause it to absorb the liquid, introducing a layer of coarse moist cement over the dry cement, and subjecting the whole to pressure.
3. The method of making tiles in a mold having bottom and removable side walls that comprises successively lubricating the bottom wall of a mold with a lubricant comprising a grease-absorbing element and an element for preventing the formation of cracks in the surface of the completed tile, positioning a pattern upon the lubricated bottom wall with portions thereof in contact with the side walls to maintain the pattern properly positioned within the mold, pouring a film-like surface layer of differ-

ently colored liquid cements upon the lubricated bottom wall between the walls of the pattern, removing the pattern to permit the differently colored liquid cements to flow towards each other and form sharp dividing lines of demarcation, introducing a layer of fine, dry cement over the liquid cement to cause it to absorb the liquid, introducing a layer of coarse moist cement over the dry cement, subjecting the whole to pressure to produce a tile, removing the side walls of the mold, thrusting the tile sidewise off the bottom wall, and immersing the tile in water to cause the tile to absorb the water and harden properly.

4. The method of making tiles that comprises successively pouring a film-like surface layer of liquid cement upon the bottom wall of a mold, introducing a layer of fine granular cement over the liquid cement, introducing a layer of coarse cement over the layer of granular cement, and subjecting the whole to pressure.

5. The method of making tiles that comprises successively positioning a pattern upon the bottom wall of a mold, pouring a film-like surface layer of differently colored liquid cements upon the bottom wall between the walls of the pattern, removing the pattern to permit the differently colored liquid cements to flow towards each other and form sharp dividing lines of demarcation, introducing a layer of fine granular cement over the liquid cement, introducing a layer of coarse cement over the layer of granular cement and subjecting the whole to pressure.

In testimony whereof, we have hereunto subscribed our names this 2nd day of November, 1922.

DOMINICK D'ALESSANDRO.  
RAFFAELE PACE.